

## UNITED STATES PATENT OFFICE

2,109,306

WOOL-LIKE ARTIFICIAL FIBERS AND PROC-  
ESS OF MAKING SAME

Arthur von Weinberg, Frankfort-on-the-Main,  
 Hanns Rein, Bad Homburg v. d. H., and Otto  
 Eisenhut, Heidelberg, Germany, assignors to  
 I. G. Farbenindustrie Aktiengesellschaft,  
 Frankfort-on-the-Main, Germany

No Drawing. Application January 5, 1934, Se-  
 rial No. 705,474. In Germany January 17,  
 1933

4 Claims. (Cl. 18—54)

Our present invention relates to wool-like artificial fibers and to a process of making same.

Artificial fibers consisting (at the end of the manufacturing processes) of regenerated cellulose, that is copper silk or viscose silk, exhibit when dried in the usual manner physical and tinctorial properties other than in the wet state. For instance a copper silk which is not yet dried possesses a high affinity to substantive dyestuffs 5 and might be dyed in deep shades already at low temperatures. This affinity is, however, diminished by the usual drying processes especially when higher temperatures are used. For this reason owing to unequal drying effects unequal 10 dyeings are obtained and soft useful products result only with the addition of textile expedients when the hitherto known drying processes are used. Thereby it is proved that the usual drying operations alter essentially the properties 15 of the fibers.

We have now found that by a special drying operation (which is per se already known and used for other materials) not only the said deterioration can be avoided or diminished but that 20 also other wise the properties of the fibers are substantially changed and the goods thus treated represent a new kind of artificial fibers unknown hitherto.

In accordance with the present invention we 25 treat wet artificial fibers which are (depending on the spinning process used) freed from metallic compounds, acids or sulfur and may be bleached and washed, with organic liquids miscible with water.

Especially suitable for our present process are 30 copper silk or copper-silk like fibers. The latter may be obtained by processes different from the copper-silk process, and are distinguished in a wet state, similar to the copper-silk itself, by a 35 high affinity to substantive dyestuffs and a small affinity to basic dyestuffs.

This drying process is advantageously carried 40 out with a fibrous material newly spun, not yet being dried, with an organic liquid easy to be re- 45 covered, at a relatively low temperature, especially room temperature, and to such a degree that the treated fibers still contain the so-called molecular water usually present in commercial brands.

The new process runs in a very simple way 50 especially as some complicated operations necessary in the processes, hitherto used, that is, washing, soaping and so on, may be dispensed with and simultaneously with the drying operation

special effects may be produced by the addition of certain preparations, that is sizing matters.

The new fibers produced by our process are distinguished by a remarkable softness, a warm touch and a crepe and curly form. These properties render them similar to animal fibers such as wool or natural silk in as high a degree as unknown hitherto. They show furthermore useful values of elasticity and strength, especially a 5 favourable elasticity.

These new and useful properties of our products are obtained, as we suppose, because the water present in the wet starting fibers is removed in an exceedingly mild way without destroying, rendering sticky or otherwise injuring 10 their surface and therefore their mechanical consistency, but with maintaining their original structure.

In order to further illustrate our invention the following examples are given; but we wish it, 20 however, to be understood that our invention is not limited to the particular products or reacting conditions stated therein.

*Example 1*

Newly spun copper-silk which is entirely freed 25 from copper and acids is introduced, immediately after being centrifuged or pressed, into a sufficient amount of alcohol (say of 95% strength). Then it is taken out of the alcohol bath, advantageously centrifuged and freed from the remaining alcohol by an aftertreatment with for instance carbon tetrachloride or ether. The solvent last used is removed from the fibers by evaporation and may be recovered.

The fibers thus obtained show the aforesaid 30 properties.

In an analogous manner other liquids customary for removing water, even containing some water themselves, may be used, single or several 40 combined, simultaneously or subsequently. The solvents are advantageously used in the liquid state.

This process may be used with the same success when the fibers are continuously spun.

*Example 2*

Wet copper silk of the like state of manufacture as that used in Example 1 is treated with acetone and then with carbon tetrachloride. 50 These solvents may be applied successively or according to a counter-current process. In order to obtain special effects the last portion of the solvent may be mixed with suitable agents, for 55

instance, sizing, impregnating or other preparations.

In an analogous manner also viscose yields by a similar single or continuous process products of like favorable properties when the regenerated cellulose, as to physical properties, is rendered similar to copper silk for instance by means of the spinning operation: see "Kunstseide", by Dr. O. Faust, 4th and 5th Ed., 1931, pages 99 and 10 218.

*Example 3*

Newly spun cellulose ribbon consisting of a great number of single filaments of for instance copper silk, immediately after having passed the usual cold or hot treating baths, is pressed, centrifugated or squeezed in order to free it mechanically from water. Then it is introduced into a bath of a low content of alcohol (say 30%). 15 From the said bath the fiber bunch is introduced into further baths of an increasing concentration of alcohol. The baths may be connected by means of overflows and provided between one another with further means for squeezing or scraping off. When the material has left the 20 bath of the highest concentration of alcohol, the adhering alcohol is removed by mechanical means so that only a small remaining portion of the alcohol is to be removed by evaporation. The goods thus obtained are reeled up. As a sudden 25 shrinking is avoided by the low concentration of the first alcoholic bath, the goods exhibit especially favorable qualities.

We claim:

1. Process of manufacturing artificial fibers 30 which comprises dehydrating newly spun wet re-

generated cellulose fibers having the dyeing properties of copper silk at room temperature in several successive baths containing liquid alcohol of an increasing concentration, the dehydration being interrupted when the treated fibers still contain the so-called molecular water usually present in commercial brands. 5

2. Process of manufacturing artificial fibers which comprises dehydrating newly spun wet copper silk at room temperature in several successive baths containing liquid alcohol of an increasing concentration, the dehydration being interrupted when the treated fibers still contain the so-called molecular water usually present in commercial brands. 10

3. Wool-like artificial fibers substantially consisting of regenerated cellulose showing the dyeing properties of copper silk and being characterized by a high affinity to substantive dyestuffs and a small affinity to basic dyestuffs, which 20 fibers are distinguished by a remarkable softness, a warm feeling and a crepe or curly form which properties render them similar to animal fibers, said artificial fiber product having been produced by the process of claim 1. 15

4. Wool-like artificial fibers consisting of copper silk distinguished by a remarkable softness, a warm feeling and a crepe or curly form which properties render them similar to animal fibers, said artificial fiber product having been produced 30 by the process of claim 2. 25

ARTHUR VON WEINBERG.

HANNS REIN.

OTTO EISENHUT.

35